

May 5, 1931.

W. A. HARTLINE

1,803,800

BLOTTING MEDIUM

Filed July 26, 1928

*Fig. 1.*



*Fig. 2.*



*Fig. 3.*



William A. Hartline, INVENTOR.

Witnesses  
C. E. Churchman  
J. G. Smith

BY Richard B. Olsen

ATTORNEYS.

## UNITED STATES PATENT OFFICE

WILLIAM A. HARTLINE, OF TAMPA, FLORIDA

## BLOTTING MEDIUM

Application filed July 26, 1928. Serial No. 295,607.

This invention relates to a blotting medium and has for its object the production of a simple and efficient blotting roller which is preferably formed of an argillaceous material having a bearing spindle of illium alloy.

In the drawings:

Fig. 1 is a view partly in elevation and partly in section illustrating one form of the blotting medium embodying the invention, this form being one adapted for employment as an attachment to fountain pens;

Fig. 2 is a view similar to Figure 1 taken in a plane at right angles to Figure 1;

Fig. 3 is a diametric longitudinal sectional view through the blotting roller shown in Figures 1 and 2, the spindle for the roller being shown in elevation.

As shown in the drawings, the blotting medium is illustrated as in the form of a cylindrical body 1, which is provided axially with a spindle 2 which is embedded therein and projects at its ends beyond the ends of the body and is mounted in suitable bearings 3, of any desired construction, located upon the end of a fountain pen which is indicated in the drawings by the numeral 4.

In accordance with the principles of the invention, the blotting medium, may be of kaolin or other argillaceous material and preferably of a clay having approximately the following composition:

|                              | Per cent |
|------------------------------|----------|
| Silica                       | 71.52    |
| Aluminum oxide ( $Al_2O_3$ ) | 27.85    |
| Calcium oxide ( $CaO$ )      | 0.63     |
|                              | 100.00   |

40 A clay of the composition above disclosed is to be preferred although various other clays may be employed for the purpose and, in fact, the invention contemplates the employment of any argillaceous material capable of being formed to the desired shape of the blotting medium and retaining its shape.

45 Where the blotting medium is to assume the form of a roller, the argillaceous material, in powdered form, is introduced into 50 suitable dies and subjected to a pressure of

from 25 to 100 pounds per square inch, the material being subjected, at such time, to a baking temperature of from 600 to 800 degrees centigrade.

In the production of the blotting medium 55 shown in Figures 1, 2 and 3, and more particularly in the last mentioned figure, the pin 2 is suitably mounted in the mold die so that in the completed article it will occupy a position extending coincident with the 60 axis of the body.

In accordance with the invention the spindle 2 is preferably of illium, which is a complex alloy of nickel and chromium, with lesser amounts of copper, molybdenum, 65 tungsten, magnesium, iron, aluminum and silicon. This alloy is highly resistant to corrosion, being substantially unaffected by acids and has sufficient hardness to serve effectually as a spindle for embedment in the 70 argillaceous material of the roller. Furthermore the alloy is not altered through oxidation nor physically by softening, under the temperatures stated above and under which temperatures the baking operation is carried 75 out.

It has been found by actual experience that a blotting medium consisting of a compressed, baked body of argillaceous material such as that contemplated by the present invention, will be absorptive to a high degree and may be employed for an indefinite period of time in blotting, without appreciable loss of efficiency, the writing fluid being rapidly absorbed by the material and in 85 a more effective manner than in the instance of the ordinary blotting paper.

It is to be understood, of course, that various changes may be made, within the scope of what is claimed, without departing from 90 the spirit of the invention.

Having thus described my invention, what I claim is:

A blotting roller of argillaceous material having a bearing spindle of illium alloy 95 embedded axially therein.

In testimony whereof I affix my signature.

WILLIAM A. HARTLINE.